

# UNITED STATES PATENT OFFICE.

WILLARD E. CASE, OF AUBURN, NEW YORK.

## ELECTROLYTIC LIQUID FOR STORAGE-BATTERIES.

SPECIFICATION forming part of Letters Patent No. 313,053, dated March 3, 1885.

Application filed April 23, 1884. (No specimens.)

*To all whom it may concern:*

Be it known that I, WILLARD E. CASE, of Auburn, Cayuga county, New York, have invented a new and useful Improvement in Electrolytic Liquids for Storage-Batteries, of which the following is a specification.

The invention consists in a neutral electrolytic liquid for storage-batteries, consisting of a solution of zinc sulphate, containing also aluminum hydrate.

I practically apply my invention as follows: First, into a solution of zinc sulphate I introduce aluminum, preferably in the form of hydrate, using two electrodes, both of lead, or 15 respectively of lead and carbon, or other suitable materials, neither electrode, however, being of zinc. On the charging of the cell the anode is oxidized and metallic zinc is deposited on the cathode. The sulphuric acid lib- 20 erated on the deposit of the zinc combines with the aluminum hydrate in the solution, forming aluminum sulphate, which is a soluble salt. The solution, being kept normal, prevents the local action of the zinc on the cathode, thus 25 saving the necessity of amalgamating the zinc and of the lead peroxide on the anode. On discharge of the cell the sulphuric acid of the aluminum sulphate attacks the zinc deposited

on the cathode, forming again zinc sulphate, and aluminum hydroxide or hydrate is liberated at the anode. This hydrate not being caustic, does not affect the lead peroxide in the anode, and is itself precipitated in the solution, when the original conditions are regained. The amount of aluminum hydrate to be added will of course depend upon the quantity of zinc deposited or acid set free from the zinc-sulphate solution. Such a quantity should be used as will at least furnish enough aluminum to satisfy the affinity of the liberated sulphuric acid, and an excess may be employed without injury. Any chemist knowing the atomic weights of the elements entering into the reactions can easily determine the proper proportion of aluminum to produce the desired result.

I claim as my invention—

In a secondary or storage cell, and in combination with the electrodes thereof, neither of said electrodes being of zinc, an electrolytic liquid normally containing zinc sulphate and aluminum hydrate, substantially as described.

WILLARD E. CASE.

Witnesses:

W. A. FRENCH,  
F. W. SMITH.